

Patented May 11, 1926.

1,584,352

# UNITED STATES PATENT OFFICE.

DAVID BELAIS, OF NEW YORK, N. Y., ASSIGNOR TO DAVID BELAIS, INCORPORATED,  
A CORPORATION OF DELAWARE.

## WHITE GOLD.

No Drawing. Application filed April 30, 1921, Serial No. 465,776. Renewed September 30, 1925.

My invention relates to the production of an improved substitute for platinum. The object of my invention is to produce a composition of matter known as white gold that will have the appearance of platinum and that may be used as a substitute for it, especially in the jewelry trade, and to produce a white gold for this purpose that will have more nearly the appearance of platinum, and that will be more malleable and ductile than any white gold previously used for this general purpose. It consists of the novel product hereinafter described and claimed.

As is well known, platinum has always been a rare metal and an expensive one, and in recent times it has become more and more so, until now the supply is wholly insufficient to meet the demand and the expense has become practically prohibitive. As is well known, platinum is peculiarly well adapted for certain uses, especially in the jewelry art, such as the setting of diamonds, the ornamentation of watch cases, and similar uses. Attempts have been made to produce a white gold that has more or less the appearance of platinum and more or less of the characteristics of platinum, among them the white gold disclosed in the patent granted to applicant, No. 1,330,231, February 10, 1920. While the article disclosed in my said patent is well adapted for such use, I have discovered a new and improved alloy which is still better adapted for the purpose, which is of a still whiter color and one more nearly corresponding with that of platinum, and that is still more malleable and ductile, and therefore better suited for the purpose. My improved alloy herein described and claimed is better adapted for use as a substitute for platinum for jewelry purposes than any heretofore known, not only because of its whiter color but because it is so much more malleable and ductile than any white gold heretofore known or used, that it can be fashioned into certain forms of jewelry not heretofore possible with any other white gold of which I am aware, for example, the fash-  
ioning into watch cases. The cost of its ingredients and the process of producing it is relatively very small compared to the cost of the platinum.

In preparing my improved alloy, I take

gold, especially or preferably fine gold, 55 nickel, preferably pure nickel, and zinc, preferably pure zinc, and a small proportion of manganese, preferably pure manganese, and fuse them together in a suitable crucible, thoroughly mixing them together 60 while they are thus fused. The resulting composition has the extremely white appearance of platinum and is especially adapted to be used as a substitute for it, as already stated. The composition is then 65 prepared for the market by being rolled or hammered into plates, wires, or other forms of commercial use, when it is ready for the trade. I use a major part of fine gold, lesser parts of nickel and zinc, and 70 a still less proportion of manganese. I have found that satisfactory results can be obtained when the gold is used in the proportion of about seventy-five (75) percent to eighty-five (85) percent, the nickel in the 75 proportion of about ten (10) percent to eighteen (18) percent, zinc in about the proportion of two (2) to nine (9) percent, and manganese in the proportion of about one-half (1/2) to two (2) percent. 80

What I claim as new and desire to secure by Letters Patent is:

1. As a composition of matter, a white gold alloy composed of a major part of gold, lesser proportions of nickel and zinc, 85 and a very small proportion of manganese.
2. As a composition of matter, a white gold alloy composed of a major part of gold, a lesser proportion of nickel, a still lesser proportion of zinc, and a still less 90 proportion of manganese.
3. As a composition of matter, a white gold alloy composed of gold, nickel, zinc, and manganese, the proportion of gold ranging from seventy-five (75) to eighty- 95 five (85) percent, the nickel from ten (10) to eighteen (18) percent, the zinc from two (2) to nine (9) percent, and the manganese from one-half (1/2) to two (2) percent.
4. A white gold alloy containing a pre- 100 ponderating amount of gold, together with relatively low percentages of nickel and zinc and a still less percentage of manganese.

In testimony whereof, I have signed my 105 name to this specification.

DAVID BELAIS.